# EUROPEAN PATENT SPECIFICATION

(11) **EP 0 118 191 B1**
(45) Date of publication and mention of the grant of the patent: **15.07.1987**
(21) Application number: 84300542.2
(22) Date of filing: 30.01.1984
(51) Int. Cl.: C11D 17/04

(54) **Laundry additive compositions**
Wäschezusatzzusammensetzungen
Compositions additives pour le linge

(30) Priority: 03.02.1983 GB 8302980
(43) Date of publication of application: 12.09.1984
(73) Proprietor: THE PROCTER & GAMBLE COMPANY, Cincinnati Ohio 45201 (US); Procter & Gamble Limited, Gosforth Newcastle upon Tyne NE99 1EE (GB)
(72) Inventor: Ingram, Barry Thomas, Whitley Bay Tyne & Wear (GB); Broughton, Paul Howard, Fenham Newcastle upon Tyne, 5 (GB)
(74) Representative: Gibson, Tony Nicholas

## Description

This invention relates to laundry additive products in the form of sheet substrates coated or impregnated with solidified detergent compositions, and is especially concerned with the separation of the solid impregnating and/or coating medium from the substrate during its passage through the processing equipment.

Laundry additive products in impregnated or coated sheet substrate form are known in the art, being disclosed in e.g. British Patent Specification Nos. 1,586,769, 2040983 and European Patent Application Nos. 0013450 and 0098129 the latter published 11.01.84. The compositions forming the coating or impregnating media for these products are primarily organic in nature and are arranged to be solid at ambient temperatures whilst being releasable from the substrate by dissolution, melting, or abrasion when added to an aqueous laundry liquor. The products are also characterised by a high loading factor, i.e. a weight ratio of coating or impregnating medium to substrate of ,3:1 so that the physical characteristics of the solidified coating or impregnating medium itself have to be taken into account in the handling of the coated or impregnated substrate, particularly when continuous manufacture of the product takes place.

Continuous manufacture of a sheet substrate product of this type involves the processing of a moving web of material, and necessitates sliding and rolling contact between the coated web and portions of the equipment. Under certain conditions it has been found that separation of the coating medium from the sheet substrate can occur, particularly at points where the coated product experiences an abrupt change of direction e.g. where the moving web separates from the contact surface. This separation manifests itself as a flaky deposit on equipment and is undesirable from a number of standpoints, as it is wasteful of coating medium, is unsightly and may affect the fuctioning of the equipment. A need therefore exists for a processing aid which will prevent or minimise this separation from the substrate of normally solid organic coating or impregnating compositions.

The use of normally solid organic processing aids is disclosed in the above mentioned British Patent Specification Nos. 1,586,769 and 2040983 but these materials, whilst satisfactory in assisting the coating and/or impregnation of flexible sheet substrates, such as non woven textile webs, have not been found useful in preventing or minimising the flaking of product from such webs or the deposit of the separated product on processing equipment.

Surprisingly, the Applicants have now found that low levels of certain liquid polyols are useful in preventing the flaking of compositions from flexible substrates in detergent additive products of the type disclosed in the above mentioned British Patent Specifications. This reduction in flaking is particularly noticeable when coated substrate products incorporating the invention are exposed to sudden angular deflection as in folding or movement around small diameter rolls.

According to the present invention there is provided a laundry additive product comprising a normally solid detergent composition comprising a solid matrix having a melting point greater than 30°C and less than 80°C, in which matrix is dispersed solid particles of size >150 pm, said solid particles comprising from 5% to 50% by weight of the composition, said composition being in water releasable combination with a flexible sheet substrate, the weight ratio of said composition to said substrate lying in the range from 1:2 to 12:1 wherein said composition includes a liquid processing aid selected from polyols of MWt ,180 and boiling point (at atmospheric pressure) of at least 100°C in an amount of from 0.5% to 5.0% by weight of the composition.

Preferably, the liquid polyols display a solubility of less than 0.1 % by weight in non polar solvents such as hexane and benzene and preferably also the liquid polyols display a high solubility in water. Most preferably the liquid polyols are completely miscible with water. The invention finds its greatest utility in those products which have a high loading factor i.e. those in which the weight ratio of the composition to the substrate is greater than 1:1, more preferably from 2:1 to 10:1, most preferably from 3:1 to 8:1.

In the context of the present invention, a material is defined as normally solid if a block of the material is self supporting at a temperature of 30°C and below. For the purposes of this invention the term 'water- releasable combination' is taken to mean a combination capable of being separated by water through solution, dispersion, leaching, softening or melting.

The laundry additive products of the present invention comprise a detergent composition of defined characteristics in water releasable combination with a flexible sheet type substrate.

The detergent composition useful in the present invention include those exemplified in British Patent Specifications Nos. 1,586,769 and 2040983 which relate to compositions comprising an organic peroxy acid bleach precursor (so-called bleach activator) in water releasable combination with a flexible sheet substrate. Mixtures of nonionic and cationic surfactants as well as peroxy acid bleach precursors are a highly preferred components of compositions of the present invention.

In the laundry additive products of the present invention the substrate is preferably absorbent and the composition is impregnated therein. Impregnation can be carried out in any convenient manner and many methods are known in the art, such as application as a solution or dispersion from an organic solvent followed by volatilisation of the solvent. However, the preferred method is by forming a melt of those components having a melting point below 100°C, dispersing the remainder of the components in the melt, applying this melt to the substrate and cooling the impregnated substrate to provide the final product.

Coated sheet products of this type, particularly when manufactured on continuous processing equipment, are prone to suffer separation of the coating from the substrate. This separation normally manifests itself as a flaky/dusty deposit on surrounding equipment and suraces and most frequently occurs when the coated product undergoes abrupt changes of orientation e.g. around small diameter rolls or in apparatus designed to fold the coated substrate. The severity of the problem is a function of many variables, such as the nature of the coating material, the absorbent capacity and physical form of the substrate, the weight of coating being applied and the stresses to which the coated substrate is subjected.

It has now been found that this flaky deposit can be prevented or considerably reduced by the inclusion in the detergent composition forming the coating impregnating medium of a liquid polyol processing aid of Molecular weight ;180 and boiling point >100°C at atmospheric pressure, in an amount of from 0.5% to 5.0% by weight of the composition, preferably from 0.5% to 3.0% by weight. Suitable polyols include glycerol and mono Cₗ-C₄ alkyl ethers and esters thereof, diethylene glycol, 1,2 propane diol and 2-methyl propane 1,2-diol. Preferred materials are glycerol and diethylene glycol.

Whilst the mechanism of the beneficial effect provided by the liquid polyols is not fully understood, it is believed that it involves a modification of the composition of the particulate solid and solidified liquid phases that result when the detergent composition is solidified after the coating and impregnation step.

The potential suitability of polyols for preventing flaking can be gauged by a screening test method which simulates the stress on coated substrates that is likely to be encountered during manufacture. The test method involves weighing the product lost and assigning a 'flaking grade' on the basis of the value obtained.

In the method a standard product is used which comprises a non woven apertured rayon sheet of basis weight 35 g/m² and size 350 mm x 230 mm impregnated with a composition comprising:

The Test method uses the following:
1 Gallenkamp shaker plus clamps
1 Glass lined open-ended vessel - height 400 mm, length 250 mm, width 100 mm
1 sheet of black card - length 250 mm, width 100 mm
1 digital balance accurate to 0.01 g
1 sheet of coated/impregnated product

### Procedure

Weigh the black card accurately on the digital balance and record. Set up the tank below the clamps on the shaker and place the black card on the base of the tank. Clamp the sheet to the shaker. Switch on the machine at its minimum setting for 1 minute, collecting all the flake falling off the sheet on the black card. Weigh the card plus flake accurately on the digital balance and record and deduct the initial card weight from the card plus flake weight.

Flaking grades are assigned on a 1-10 scale as follows, the higher numbers donating improvement in flaking grade. Product having a flaking grade <5 is regarded as unsatisfactory.

On this basis various materials graded as follows:

Preferred materials are glycerol and diethylene glycol used in amounts of 0.1-0.3 g/sheet, corresponding to a range of from 0.5% to 1.6% based on the weight of the detergent composition.

The detergent composition is normally solid i.e. can be formed into a body which is self supporting at temperatures of 30°C and below. It is composed of a solidifed liquid mass, which has a melting point lying between 30°C and 80°C in which are dispersed solid particles of size <150 pm, preferably <50 itm.

The detergent composition comprises any of the conventional functional components normally used in laundry detergents such as surfactants of anionic, nonionic, cationic amphoteric or zwitterionic type, suds modifiers, detergent builder salts, chelating agents, peroxygen bleaches, organic peroxy bleach precursors, anti-redeposition agents, antibacterial agents, fabric softening and antistatic agents, optical brighteners, anticorrosion agents, enzymes, perfumes, dyes and pigments.

Most of the above components, if present in the additive product of the invention, form the solid particulate phase which may be organic or inorganic in type or may be a mixture of the two. Certain components such as nonionic surfactants, suds modifiers and certain anti-redeposition agents are solids having melting points within the temperature range required for the solidified liquid mass and so can be employed both as functional components and as carriers for the remainder.

With respect to the surfactants, those of anionic type can be natural or synthetic in origin whilst nonionic surfactants can be either semi-polar or alkylene oxide condensates. Examples of each of these classes of compounds are disclosed in Laughlin & Heuring US Patent No. 3,929,678 issued 30 December 1975. Cationic surfactants can include amine salts, quaternary nitrogen and phosphorus compounds and ternary sulphonium compounds. The invention is particularly useful in additive products incorporating a quaternary ammonium surfactant as the or part of the solid particles.

The nonionic surfactants used in the compositions may be alkoxylated aliphatic alcohols, alkyl phenols, esters, amides and fatty acids having an HLB within the range 8.0-17.0. The aliphatic alcohols include linear and branched chain primary and secondary Cₐ₋C₂₂ alcohols, the alkyl phenols are the C₆―C₁₂ alkyl phenols, and the fatty esters, fatty amides and fatty acids are those having a C₁₂―C₁₈ alkyl group in the acyl residue. The preferred alkoxylating group is ethylene oxide.

Suitable nonionic surfactants based on aliphatic alcohols are condensation products of primary and secondary alcohols with from 4 to 30 moles of ethylene oxide. The alkyl chain of the aliphatic alcohol can either be straight or branched and generally contains from 8 to 22 carbon atoms. Examples of such ethoxylated alcohols include the condensation product of myristyl alcohol with 10 moles of ethylene oxide per mole of alcohol and the condensation product of 9 moles of ethylene oxide with coconut alcohol (a mixture of fatty alcohols with alkyl chains varying in length from 10 to 14 carbon atoms). Examples of nonionic surfactants of this type include those commercially available under the Trade Names Tergitol 15-S-9, marketed by Union Carbide Corporation, Neodol 45E9, marketed by Shell Chemical Company, and Kyro EOB, marketed by The Procter & Gamble Company. Other suitable alcohol ethoxylates include:-

Alcohol ethoxylates such as those disclosed in British Patent Specification No. 1,462,134 are also useful.

Suitable alkyl phenol ethoxylates include the condensation products of alkyl phenols having an alkyl group containing from 6 to 12 carbon atoms in either a straight chain or branched chain configuration with ethylene oxide, said ethylene oxide being present in an amount equal to 8 to 20 moles of ethylene oxide per mole of alkyl phenol. The alkyl substituent in such compounds can be derived, for example, from polymerized propylene, di-isobutylene, and the like. Examples of compounds of this type include nonyl phenol condensed with 9.5 moles of ethylene oxide per mole of nonyl phenol; dodecylphenol condensed with 12 moles of ethylene oxide per mole of phenol; and di-isooctyl phenol condensed with 15 moles of ethylene oxide per mole of phenol. Nonionic surfactants of this type include those commercially available under the trade names Igepal CO-630, marketed by the GAF Corporation, and Triton X-45, X-114, X-100, and X-102, all marketed by the Rohm & Haas Company.

Other suitable phenol ethoxylates include:-

Suitable fatty acid ethoxylates include coconut fatty acid (E₅) and oleic fatty acid (Eₗₒ), while ester ethoxylates include:

Other nonionic surfactants useful herein include the condensation products of ethylene oxide with the product resulting from the reaction of propylene oxide and ethylene diamine, and the condensation product of ethylene oxide with the product resulting from the condensation of propylene oxide with propylene glycol. Surfactants of this type are available commercially from the Wyandotte Chemicals Corporation under the Registered Trade Marks "Tetronic" and "Pluronic" respectively.

Particularly preferred nonionic surfactants as components of the compositions useful in the present invention are the primary linear and branched chain primary alcohol ethoxylates, such as C,₄-C,₅ linear alcohols condensed with 7-15 moles of ethylene oxide available from Shell Oil Co. under the Trade Name "Dobanol" and the C₁₆―C₁₃ branched chain alcohol ethoxylates obtainable from Liquichimica SA under the Trade Name "Lial". The cationic surfactants forming preferred components of the compositions useful in the present invention have the empirical formula

wherein each R' is a hydrophobic organic group containing alkyl chains, alkenyl chains, alkyl benzyl chains, alkyl phenyl chains, ether linkages, alkylene groups, alkenylene groups, ester linkages, or amide linkages totalling from 8 to 22 carbon atoms and which may additionally contain or be attached to a polyethylene oxide chain containing up to 20 ethoxy groups, m is a number from one to three provided that no more than one R' in a molecule can have more than 16 carbon atoms when m is 2 and no more than 12 carbon atoms when m is 3, R² is an alkyl or hydroxyalkyl group containing from 1 to 4 carbon atoms or a benzyl group, with no more than one R² in a molecule being benzyl, and x is a number from 1 to 3, Y is selected from and Z is a water-soluble anion selected from halide, methosulphate, carboxylate, hydroxide, or nitrate, particularly preferred being chloride, bromide or iodide anions, in a number to give electrical neutrality of the cationic component. The particular cationic component to be included in a given system depends to a large extent upon the particular nonionic component to be used in this system, and is selected such that it is at least water-dispersible, or preferably water-soluble, when mixed with said nonionic surfactant. It is preferred that the cationic component be substantially free of hydrazinium groups. Mixtures of these cationic materials may also be used in the compositions of the present invention.

When used in combination with nonionic surfactants, these cationic components provide excellent soil removal characteristics, confer static control benefits to the laundered fabrics, and inhibit the transfer of dyes among the laundered fabrics in the wash solution.

In preferred cationic materials, L is equal to 1 and Y is However, L may be greater than 1, such as in cationic components containing 2 or 3 cationic charge centres.

Where Y is and m = 1, it is preferred that x is equal to 3. R₂ is normally a methyl group but a preferred structure is where one R₂ group is hydroxy ethyl. Cationic surfactants of this mono long chain type include those in which R' is a C₁₀―C₁₀ alkyl group more preferably a C₁₀―C₁₆ alkyl group. Particularly preferred compositions of this class include C₁₂ and C₁₄ alkyl trimethyl ammonium bromide, C₁₂ alkyl dimethyl hydroxy ethyl ammonium bromide and C₁₂ alkyl dimethyl hydroxypropyl ammonium bromide and their counterparts based on middle-cut coconut alcohol as the source of the alkyl group. Other counter ions such as methosulphate and carboxylate can also be used particularly with the hydroxyalkyl-substituted compounds.

When m is equal to 2, only one of the R' chains should be longer than 16 carbon atoms. Thus, ditallow- dimethylammonium salts used conventionally as fabric softeners and static control agents in detergent compositions, are unsuitable as the cationic component in surfactant mixtures. Preferred di-long chain cationics of this type include those in which x is equal to 2 and R² is a methyl group. Particularly preferred cationic materials of this class include are those in which R, is C₈―C₁₂ alkyl such as the di-Cₐ alkyl dimethylammonium salt, the di-C₁₀ alkyldimethylammonium salts and the di-C₁₂ alkyldimethylammonium salts materials.

Where m is equal to 3, only one of the R' chains can be greater than 12 carbon atoms in length. The reason for this chain length restriction, as is also the case with the di-long chain cationics described above, is the relative insolubility of these tri- and di-long chain materials. Where tri-long chain alkyl materials are used, it is preferred that x is equal to 1 and that R² is a methyl group. In these compositions it is preferred that R' is a C₈ to C₁₁ alkyl group. Particularly preferred tri-long chain cationics include trioctylmethylammonium halide, and tridecylmethylammonium halide.

Cationic components in which m is equal to 1 and the hydrophobic group R, is interrupted by ester linkages are disclosed in US-A-4260529. Particularly preferred cationic surfactants of this type are the choline ester derivatives having the following formula as well as those wherein the ester linkage in the above formula is replaced with a reverse ester, amide or reverse amide linkage.

Particularly preferred examples of this type of cationic surfactant include stearoyl choline ester quaternary ammonium halide (R³ = C₁₇ alkyl), palmitoyl choline ester quaternary ammonium halides (R³ = C₁₆ alkyl), myristoyl choline ester quaternary ammonium halides (R³ = C₁₃ alkyl), lauroyl choline ester ammonium halides (R³ = C" alkyl), and tallowoyl choline ester quaternary ammonium halides (R³ = C₁₆―C₁₈ alkyl).

The above described cationic components are useful in nonionic/cationic surfactant mixtures which have a ratio of nonionic to cationic of from 1:2 to 20:1. Preferably, nonionic to cationic ratios of from 10:1 to 1:1 are used, more preferably from 5:1 1 to 3:2, most preferably from 10:3 to 10:5. These cationic surfactants may also be used in the detergent systems defined in US Patent No. 4,259,217, in nonionic to cationic ratios of from 8:1 to 20:1.

In compositions incorporating mixtures of nonionic and cationic surfactants it is preferred that the amount of the nonionic-cationic mixture is such that the surfactant mixture:substrate weight ratio lies in the range 10:1 to 1:5, preferably from 10:1 to 1:2, and most preferably from 5:1 to 1:1. In preferred executions using non-woven sheet substrates of approximately 805 _{CM}² plan area and 3 grs/sheet basis weight, the loading of nonionic-cationic surfactant mixture is in the range 5-15 grs/sheet.

Suds modifiers useful in the detergent compositions can be of the suds boosting, suds stabilising or suds suppressing type. Examples of the first type include the C₁₂-C₁₈ fatty acid amides and alkanolamides, the second type is exemplified by the C_{'2}-C_{'6} alkyl dilower alkyl amine oxides and the third type by C₂₀-C₂₄ fatty acids, certain ethylene oxide-propylene oxide copolymers such as the "Pluronic" series, silicones, silica-silicone blends, micro-crystalline waxes, triazines and mixtures of any of the foregoing.

Preferred suds suppressing additives are described in US Patent 3,933,672, issued January 20, 1976, relative to a silicone suds controlling agent. The silicone material can be represented by alkylated polysiloxane materials such as silica aerogels and xerogels and hydrophobic silicas of various types. The silicone material can be described as siloxane having the formula: wherein x is from 20 to 2,000, and R and R' are each alkyl or aryl groups, especially methyl, ethyl, propyl, butyl and phenyl. The polydimethylsiloxanes (R and R' are methyl) having a molecular weight within the range of from 200 to 200,000, and higher, are all useful as suds controlling agents. Additional suitable silicone materials which exhibit useful suds controlling properties, are those wherein the side chain groups R and R' are alkyl, aryl, or mixed alkyl and aryl hydrocarbyl groups, examples including diethyl-, dipropyl-, dibutyl-, methyl-, ethyl-, and phenylmethylpolysiloxanes. Additional useful silicone suds controlling agents can be represented by a mixture of an alkylated siloxane, as referred to hereinbefore, and solid silica. Such mixtures are prepared by affixing the silicone to the surface of the solid silica. A preferred silicone suds controlling agent is represented by a hydrophobic silanated (most preferably trimethylsilanated) silica having a particle size in the range from 10 nanometers to 20 nanometers and a specific surface area above 50 m²/g intimately admixed with dimethyl silicone fluid having a molecular weight in the range from 500 to 200,000 at a weight ratio of silicone to silanated silica of from 19:1 to 1:2. The silicone suds suppressing agent is advantageously releasably incorporated in a water-soluble or water-dispersible, substantially non- surface-active detergent-impermeable carrier.

Particularly useful suds suppressors are the self-emulsifying silicone suds suppressors, described in US Patent No. 4,136,045. An example of such a compound is DB-544, commercially available from Dow Corning, wich is a siloxane/glycol copolymer.

Suds modifiers as described above are incorporated at levels of up to approxiamtely 5%, preferably from 0.1 to 2% by weight of the cationic-nonionic surfactant mixture.

Detergent builder salts can be inorganic or organic in type but the crystalline nature of inorganic builder salts, and hence the difficulty of incorporating them by coating or impregnation puts constraints on the amounts which can be included in the products of the invention. This results in a practical upper limit on the weight ratio of inorganic builder to substrate of about 5:1. Organic builder salts such as citrates, mellitates, phytates, nitrilo triacetates, carboxymethyloxy succinates, polyacrylates and polyhydroxy- acrylates can be incorporated at higher levels, i.e. up to a weight ratio of builder to substrate of about 8: 1.

Chelating agents that can be incorporated include citric acid, nitrilotriacetic and ethylene diamine tetra acetic acids and the salts, organic phosphonate derivatives such as those disclosed in Diehl US Patent No. 3,213,030 issued 19 October, 1965; Roy US Patent No. 3,433,021 issued 14 January, 1968; Gedge US Patent No. 3,292,121 issued 9 January, 1968; and Bersworth US Patent No. 2,599,807 issued 10 June, 1952, and carboxylic acid builder salts such as those disclosed in Diehl US Patent No. 3,308,067 issued 7 March, 1967. Preferred chelating agents include nitrilotriacetic acid (NTA), nitrilotrimethylene phosphonic acid (NTMP), ethylene diamine tetra methylene phosphonic acid (EDTMP) and diethylene triamine penta methylene phosphonic acid (DETPMP), and these are incorporated in amounts such that the substrate chelating agent weight ratio lies in the range 20:1 to 1:5, preferably 5:1 to 1:5 and most preferably 3:1 to 1:1.

Inorganic peroxygen bleaches which can be incorporated include those which are true peroxysalts such as alkali metal monopersulphates as well as salts which include hydrogen peroxide, such as sodium perborate monohydrate and tetrahydrate, sodium percarbonate, sodium persilicate and sodium perpyrophosphate.

Clathrates such as that comprising 4Na₁SO₄: 2H₂O₁: 1 NaCl can also be incorporated provided that moisture is excluded from the compositions. Mixing of the bleach with the other components can be employed in certain instances but where materials reactive towards the bleach such as organic peroxy acid bleach precursors are included, spatial separation of the bleach from these materials is necessary.

Organic peroxy acid bleach precursors are preferred components of laundry products of the invention and any of the precursors disclosed in British Patent Specification Nos. 1,586,769 and 2040983 and European Patent Application No. 0098129, published 11.01.84, can be included. Preferred precursors include tetra acetyl alkylene diamine, in which the alkylene group can contain from 1 to 6 carbon atoms tetra acetyl glycoluril, sodium p-C,-C₉ acyloxybenzene sulphonates in which the alkyl portion of the acyl group may be linear or branched, penta acetyl glucose, octa acetyl lactose and mixtures of any of these.

Certain polybasic acids have been found to enhance the bleaching effect of organic peroxyacids, examples being EDTMP, NTMP and DETPMP. However, not all chelating polybasic acids are useful in this respect, while certain poorly-chelating polybasic acids, notably succinic acid, and glutaric acid, do show efficacy.

The level of usage of the precursor will naturally be dependent on a number of factors e.g. the size of the fabric load in the machine, the level of bleaching performance desired, the amount of perhydroxyl ion in the wash solution, the bleaching efficacy of the organic peroxy species derived from the precursor and the efficiency of conversion of the precursor into that peroxy species. It is conventional with inorganic peroxy bleaches to provide a level of available oxygen in solution from 50 ppm to 350 ppm by weight for heavy duty laundry purposes. However, when using organic peroxy bleaches a level of available oxygen provided by the organic peroxy compound may lie in the range from 2 ppm to 100 ppm, levels of from 3 ppm to 30 ppm being appropriate under conventional US washing conditions while levels of from 20 ppm to 50 ppm are more commonly used under European washing conditions. This level of available oxygen should be attained within the normal wash cycle time i.e. within 5-25 minutes depending on the particular wash cycle being employed.

For a machine having a liquid capacity in use of 20 to 30 litres, such a level of available oxygen requires the delivery of from 1 gr to 20 gr of organic peroxy compound precursor assuming quantitative conversion. Preferably a single unit of substrate should be capable of accommodating the desired level of precursor and any adjuvants and additives that it is necessary to incorporate into the product, although the number of units to be used to deliver a given quantity of precursors is a matter of choice. Normally the weight of precursor per delivery will lie in the range 3 to 10 grs, preferably from 4 to 6 grs.

Anti redeposition and soil suspension agents also constitute preferred components of the additive compositions of the invention. Cellulose derivatives such as methyl cellulose, carboxymethyl cellulose and hydroxy ethyl cellulose are examples of soil suspension agents and suitable antiredeposition agents are provided by homo- or co-polymeric polycarboxylic acids or their salts in which at least two carboxyl radicals are present separated by not more than two carbon atoms. Polyethylene glycols of MWt 1,000-10,000 particularly of MWt 4,000-10,000 are also useful particulate soil suspension agents and function as such even if included primarily as processing aids.

Highly preferred polymeric polycarboxylic acids are copolymers of maleic acid or maleic anhydride with methyl vinyl ether, ethyl vinyl ether or acrylic acid, the polymers having a molecular weight in the range from 12,000 to 1;500,000.

A further description of suitable polymeric polycarboxylic acids is provided in the Applicants' European Patent Application Publication No. 63017. Levels of incorporation of these antiredeposition agents are such as to provide agent:substrate ratios of 2:1 to 1:20, preferably 1:2 to 1:10.

Suitable antibacterial agents are quaternary ammonium compounds such as cetyl pyridinium chloride, cetyl trimethyl ammonium bromide and C₈-C,₈ alkyl benzyl dimethyl ammonium chloride, typically incorporated in weight ratios of agent to substrate of from 1:1 to 1:10.

A wide range of fabric softeners and antistatic agents can be included as optional compounds. Exemplary cationic nitrogen compounds include the di-C,₆-C,₈ alkyl, di-C,-C₄ alkyl quaternary ammonium salts, imidazolinium salts and non-nitrogenous materials such as the sorbitan esters of C₁₆―C₁₈ fatty acids. These are normally incorporated at softener to substrate weight ratios of 5:1 to 1:1.

Optical brighteners may be anionic or nonionic in type and are added at levels of from 0.05 to 1.0 grs per sheet preferably 0.1 to 0.5 grs per sheet.

Anionic fluorescent brightening agents are well-known materials, examples of which are disodium 4,4'-bis-(2-diethanolamino-4-anilino-s-triazin-6-ylamino) stilbene-2:2'-disulphonate, disodium 4,4'-bis-(2-morpholino-4-anilino-s-triazin-6-ylamino)stilbene-2:2'-disulphonate, disodium 4,4'-bis-(2,4-dianilino-s-triazin-6-ylamino) stilbene-2:2'-di-sulphonate, disodium 4,4'-bis-(2-anilino-4-(N-methyl-N-2-hydroxyethyl- amino) stiibene-2,2'-di-suiphonate, disodium 4,4'-bis-(4-phenyl-2,1,3-triazol-2-yl)-stilbene-2,2'- disulphonate, disodium 4,4'-bis(2'-anilino-4-(1-methyl-2-hydroxyethylamino)-s-triazin-6-ylamino)stilbene-2,2'-disulphonate, sodium 2(stilbyl-4"-(naptho-1',2':4,5)-1,2,3-triazol-2"-sulphonate and di-sodium 4,4'- bis(2-sulphonato styryl)biphenyl.

Other fluorescers to which the invention can be applied include the 1,3-diaryl pyrazolines and 7-alkyl- aminocourmarins.

A preferred fluorescer is the anionic material available from Ciba Geigy S.A. under the trade name Tinopal (RTM) CBS and mixtures thereof with materials available under the trade names Tinopal (RTM) EMS and Blankophor (RTM) MBEN, the latter being sold by Farbenfabriken Bayer AG.

Other preferred optional ingredients include the multifunctional photoactivator/dyes belonging to the porphine class of general formula wherein each X is (=N-) or (=CY-), and the total number of (=N-) groups is 0, 1, 2, or 4; wherein each Y, independently, is hydrogen or meso substituted alkyl, cycloalkyl, aralkyl, aryl, alkaryl or heteroaryl; wherein each R, independently, is hydrogen or pyrrole substituted alkyl, cycloalkyl, aralkyl, aryl, alkaryl or heteroraryl, or wherein adjacent pairs of R's are joined together with orthoarylene groups to form pyrrole substituted alicyclic or heterocyclic rings; wherein A is 2(H) atoms bonded to diagonally opposite nitrogen atoms, or Zn(II), Cd(II), Mg(II), Ca(II), AI(III), Sc(lll), or Sn(IV); wherein B is an anionic, nonionic or cationic solubilizing group substituted into Y or R; wherein M is a counterion to the solubilizing groups; wherein, when B is cationic, M is an anion and s is from 1 to 8; when B is nonionic, B is polyethoxylate, M is zero, s is from 1 to 8, and the number of condensed ethylene oxide molecules per porphine molecule is from 8 to 50; when B is anionic and proximate, M is cationic and s is from 3 to 8; when B is anionic and remote, M is cationic and s is from 2 to 8; and when B is sulphonate the number of sulphonate groups is no greater than the number of aromatic and heterocyclic substituent groups.

As used herein, a solubilizing group attached to a carbon atoms displaced more than 5 carbon atoms away from the porphine core is referred to as "remote"; otherwise it is "proximate".

Highly preferred materials of this general type are the zinc phthalocyanine tri- and tetrasulphonates and mixtures thereof. Materials of this general class were originally disclosed for use in detergent compositions in British Patents 1,372,035 and 1,408,144 and are discussed in detail in European Patent Application 3861. The photo-activators can provide bleaching effects on fabrics washed with the detergent additive compositions and dried in the presence of visible light and atmospheric oxygen and can also synergistically enhance the bleaching effect of conventional bleaching agents such as sodium perborate. The porphine bleach is preferably used in an amount such that the level of porphine in the composition is in the range from 0.004% to 0.5%, more preferably from 0.001 % to 0.1 %, especially from 0.002% to 0.05% by weight.

Preferred enzymatic materials include the commercially available amylases, and neutral and alkaline proteases conventionally incorporated into detergent compositions. Suitable enzymes are discussed in US Patents 3,519,570 and 3,533,139. Examples of suitable enzymes include the materials sold under the Registered Trade Marks Maxatase, Rapidase and Alcalase.

As stated previously most of the above-mentioned functional ingredients, with the exception of the nonionic surfactants, the organic suds modifiers and certain anti-redeposition agents, are solid materials which form the dispersed particulate phase of the detergent compositions. The particulates are insoluble, or only partly soluble, in the solidified liquid phase and ideally are finely divided. Their particle size is of no more than 150 µm and preferably should be less than 100 µm, ideally less than 50 pm.

Preferred detergent compositions useful in the present invention include one or more of a cationic surfactant as hereinbefore defined, most preferably of the type where Y is I and m is 1 or 2, a chelating agent of the amino polyphosphonate type particularly EDTMP or DETPMP and a peroxyacid bleach precursor of the tetracetyl alkylene diamine and/or Cₗ-Cg acyloxybenzene sulphonic or carboxylic acid type, together with a C₈-C₂₂ ethoxylated primary alcohol and a polyethylene glycol of MWt 4,000-10,000.

The types and levels of the ingredients of the detergent composition is constrained by the requirements of mutual unreactivity (if the materials are applied so as to be in intimate contact), by the weight ratio of components forming particulate solids to components forming the solidified liquid phase and by the loading limitations of the substrate. As mentioned above, materials that are capable of mutual reaction can be incorporated in the additive products of the invention, but must be spatially separated from each other i.e. by application to a substrate location that is free or substantially free of the other reactant material(s). The detergent composition is preferably applied, as described in more detail hereinafter, as a molten dispersion to the substrate so that the maximum viscosity that can be handled by the application system determines the maximum level of dispersed particulate solids in the composition. This level is 50% by weight. The minimum level of 5% by weight of the composition is less critical. Preferably the level of dispersed particulate solids is from 25% to 45% by weight of the composition.

Within the limits imposed by the ratio of particulate solid to solidified liquid components, individual components can be incorporated in amounts up to those corresponding to component:substrate weight ratios of 10:1. However, for processing and product aesthetics reasons, the total weight of particulate components per sheet is normally held to a maximum of 4 times the sheet weight, and individual components are ideally present at no more than 3 times the sheet weight.

The detergent compositions useful in the invention also comprise a solidified liquid phase in which the solid particles are dispersed. As mentioned above certain functional components of the composition such as nonionic surfactants can act as the, or part of the, solidified liquid phase but in general the majority of the solidified liquid phase is a water soluble or water dispersible processing aid having a melting point in the range from 30°C to 80°C. The most preferred processing aids are organic compounds having a softening point greater than 40°C and a melting point less than 80°C to permit their easy processing.

These compounds serve as an aid in processing and/or in releasing the compostion from the substrate when the latter is introduced into a wash liquor and, when melted, provide mixtures having a viscosity of up to 5000 mPa.s at 50°C.

Typical solids are C₁₄―C₁₈ primary and secondary alcohols and C,₂₇-C₂₀ fatty acids and ethoxylates thereof containing from 15 to 80 ethylene oxide groups per mole of alcohol, sorbitan esters of C₁₂―C₂₀ fatty acids and polyethylene glycols of Mwt 4000-10,000. Insoluble waxy materials such as paraffin waxes and alkyl fatty acid esters can also be used in minor amounts in admixture with one or more water soluble materials. Mixtures of the above water soluble materials are preferred.

As indicated above, the organic compounds forming the solidified liquid phase can serve as a release aid that assists in releasing the compositions from the substrate upon addition of the product to a wash liquor. In general, materials serving as processing aids are also suitable as release aids but certain materials, notably C,₆-Cₗ. fatty acids and polyethylene glycols of MWt 4,000-10,000, are particularly effective when used in amount such that the weight ratio of compositions: release aid lies in the range 9:1 to 1:1 particularly 3:1 to 1:1.

It will be apparent that the detergent compositions of the additive products in accordance with the invention will incorporate a high level of organic material having a Mpt> 30°C and this will include at least 50% by weight of the composition of carrier material having a melting point in the range 30°C80°C either in the form of a processing aid or as one of the functional detergent components. Typically the composition will incorporate at least 55% of such carrier materials and, depending on the nature and physical characteristics of the "non-carrier" solid components, the level of carrier materials may be as high as 70% of the composition.

The substrate may itself be water soluble or water insoluble and in the latter case if should preferably possess sufficient structural integrity under the conditions of the wash to be recovered from the machine at the end of the laundry cycle. Water soluble materials include certain cellulose ethers, alginates, polyvinyl alcohol and water soluble polyvinyl pyrrolidone polymers, which can be formed into non-woven and woven fibrous structures. Suitable water insoluble materials include, but are not restricted to, natural and synthetic fibres, foams, sponges and films.

Preferably the sheet is water pervious i.e. water can pass from one surface of the sheet to the opposite surface and, for film type substrates, perforation of the sheet is desirable. The most preferred form of the substrate is a sheet of woven or non-woven fabric or a thin sheet of cellular plastics material. Woven fabric sheets can take the form of a plain weave natural or synthetic fibre of low fibre count/unit length, such as is used for surgical dressings, or of the type known as cheese cloth. Loading limitations on sheet type substrates limit the amount of detergent composition that can be applied to the sheet namely to a maximum represented by a precursor:sheet weight ratio of about 10:1.

A very desirable attribute of the laundry additive products of the present invention is that they do not interfere with the mechanical operation of the washing machine into which they are put. A high proportion of domestic washing machines are of the rotating perforated drum type in which the perforations extend over the entire peripheral surface. In this type of equipment the drum construction and mode of operation obviates any problem of obstruction to liquid flow in the machine. Certain older types of machine utilise an agitator in a stationary vessel provided with a recirculating liquid system. In order to avoid liquid blockage in this machine type it may be necessary to provide slits or perforations in the substrate, particularly if it is in sheet form. Sheet structures of this type are disclosed in McQueary US Patents Nos. 3944694 and 3956556 issued March 16, 1976 and May 11, 1976 respectively.

As stated above, suitable materials which can be used as a substrate in the invention herein include, among others, sponges, paper, and woven and non-woven fabrics.

A suitable sponge like material that can be used in the present invention comprises an absorbent foam like material in the form of a sheet. The term 'absorbent foam-like material' is intended to encompass three dimensional absorptive materials such as'gas blown foams', natural sponges and composite fibrous based structures such as are disclosed in US Patent Nos. 3311115 and 3430630. A particularly suitable material of this type is a hydrophilic polyurethane foam in which the internal cellular walls of the foam have been broken by reticulation. Foams of this type are described in detail in Dulle US Patent No. 3794029. A preferred example of this foam type comprises a hydrophilic polyurethane foam of density 0.036 g/cm³ (0.596 grs per cubic inch) with a cell count of between 8 and 40 cells per cm, preferably about 24 to 32 per cm available from the Scott Paper Company, Eddystone, Pennsylvania USA., under the Registered Trade Mark "Hydrofoam". Preferred sheets of this type of material have thicknesses in the range from 3 to 5 mm.

A suitable paper-based absorbent structure containing 2 or 3 paper plies is disclosed in US-A-3414459.

The preferred substrates of the laundry additive products of the invention are apertured and non apertured nonwoven fabrics which can generally be defined as adhesively bonded fibrous or filamentous products, having a web or carded fibre structure (where the fibre strength is suitable to allow carding) or comprising fibrous mats, in which the fibres or filaments are distributed haphazardly or in random array (i.e. an array of fibres in a carded web wherein partial orientation of the fibres is frequently present as well as a completely haphazard distribution orientation) or substantially aligned. The fibres or filaments can be natural (e.g. wool, silk, wood pulp, jute, hemp, cotton, linen, sisal, or ramie), synthetic (e.g. rayon, cellulose, ester, polyvinyl derivatives, polyolefins, polyamides, or polyesters) or mixtures of any of the above.

Methods of making non-woven cloths are not a part of this invention and being well known in the art, are not described in detail herein. Generally, such cloths are made by air or water laying processes in which the fibres or filaments are first cut to desired lengths from long strands, passed into a water or air stream, and then deposited onto a screen through which the fibre-laden air or water is passed. The deposited fibres or filaments are then adhesively bonded together, dried, cured and otherwise treated as desired to form the non-woven cloth. Non-woven cloths made of polyesters, polyamides, vinyl resins, and other thermoplastic fibres can be bonded, i.e. the fibres are spun out onto a flat surface and bonded (melted) together by heat or by chemical reactions.

The absorbent properties desired herein are particularly easy to obtain with non-woven cloths and are provided merely by building up the thickness of the cloth, i.e. by super-imposing a plurality of carded webs or mats to a thickness adequate to obtain the necessary absorbent properties, or by allowing a sufficient thickness of the fibres to deposit on the screen. Any diameter or denier of the fibre (generally up to about 10 denier, 1 denier being equal to 1,1 dtex) can be used, inasmuch as it is the free space between each fibre that makes the thickness of the cloth directly related to the absorbent capacity of the cloth, and which further makes the non-woven cloth especially suitable for impregnation with a peroxy compound detergent composition by means of interstitial or capillary action. Thus, any thickness necessary to obtain the required absorbent capacity can be used.

The choice of binder-resins used in the manufacture of non-woven cloths can provide substrates possessing a variety of desirable traits. For example, the absorbent capacity of the cloth can be increased, decreased, or regulated by respectively useing a hydrophilic binder-resin, a hydrophobic binder-resin or a mixture thereof in the fibre bonding step. Moreover, the hydrophobic binder-resin, when used singly or as the predominant compound of a hydrophobic-hydrophilic mixture, provides non-woven cloths which are especially useful as substrates when the detergent composition-substrate combinations disclosed herein are used in an automatic washer.

When the substrate herein is a bonded non-woven cloth made from fibres, deposited haphazardly or in random array on the screen, the compositions exhibit excellent strength in all directions and are not prone to tear or separate when used in the washer.

Preferably, the non-woven cloth is water-laid or air-laid and is made from cellulosic fibres, particularly from regenerated cellulose or rayon, which are lubricated with standard textile lubricant. Preferably the fibres are from 4 to 50 mm in length and are from 0.16 to 0.55 Tex. Preferably the fibres are at least partially orientated haphazardly, particularly substantially haphazardly, and are adhesively bonded together with hydrophobic or substantially hydrophobic binder-resin, particularly with a nonionic self-crosslinking acrylic polymer or polymers. Conveniently, the cloth comprises 70% fibre and 30% binder-resin polymer by weight and has a basis weight of from 10 to 100, preferably from 24 to 72 g/m².

A suitable example is an air-laid, non-woven cloth comprising 70% regenerated cellulose (American Viscose Corporation) and 30% hydrophobic binder-resins (Rhoplex HA-8 on one side of the cloth, Rhoplex HA-16 on the other; Rhoplex being a Trade Name for binder resins sold by Rohm & Haas, Inc). The cloth has a thickness of 0.1 to 0.125 mm and a basis weight of 29 g/m². A 30 cm length of the cloth 21 cm wide weighs 1.78 grams. The fibers are 10 mm in length, 0.16 tex, and are orientated substantially haphazardly. The fibres are lubricated with sodium oleate.

A further exemplary substrate is a water-laid, non-woven cloth commercially available from C H Dexter Co., Inc. The fibres are regenerated cellulose, 15 mm in length, 0.16 tex, and are lubricated with a similar standard textile lubricant. The fibres comprise 70% of the non-woven cloth by weight and are orientated substantially haphazardly; the binder-resin (HA-8) comprises 30% by weight of the cloth. The substrate is 0.1 mm thick, and it has a basis weight of 29 g/m^{2.} A 30 cm length of the cloth 21 cm wide, weighs 1.66 grams.

Apertured non-woven substrates are also useful for the purposes of the present invention. The apertures, which extend between opposite surfaces of the susbtrate are normally in a pattern and are formed during lay-down of the fibres to produce the substrate. Exemplary apertured non-woven substrates are disclosed in US Patent Nos. 3,741,724, 3,930,086 and 3,750,237.

A suitable diamond patterned apertured substrate is obtainable from Chicopee Manufacturing Co., Milltown, New Jersey, USA under the Code No. SK 650 WFX 577 and comprises a polyester-wood pulp mixture have a basis weight of 50 g/m² and approximately 13 apertures per square cm.

Another preferred example of an apertured non-woven substrate, also available from Chicopee Manufacturing Co., under the Code No. AK 30 ML 1379 comprises a regenerated cellulose sheet of 3.3 dtex fibres bonded with Rhoplex RA 8 binder (fibre:binder ratio 70:30) having a basis weight of 40 g/m² and 17 apertures/cm2. A highly preferred square patterned apertured substrate of similar composition but fibre:binder ratio of 80:20 and basis weight 35 g/m² is also available from Chicopee BV Holland.

In general, apertured fabrics for the purposes of the invention have from 10-20 apertures/cm2, preferably 12-18 apertures/cm2.

The size and shape of the substrate sheet is a matter of choice and is determined principally by factors associated with the convenience of its use. Thus the sheet should not be so small as to become trapped in the crevices of the machine or the clothes being washed or so large as to be awkward to package and dispense from the container in which it is sold. For the purposes of the present invention sheets ranging in plan area from 130 cm² to 1300 _{CM}² are acceptable, the preferred area lying in the range of from 650 cm² to 900 _{cm}2_{.}

The invention is illustrated in the following examples in which all parts and percentages are by weight of the composition unless otherwise specified.

In the Examples, the abbreviations used have the following designation:

### Example 1

### The following product was prepared:

The substrate was a square patterned apertured non-woven sheet, of size 23 x 35 cm and basis weight 2.8 g, formed of 100% unbleached crimped rayon fibres (80% fibre, 20% polyacrylate binder). The product was made by forming a melt of the PEG and A 45E7 at approximately 80°C, dispersing the other components (except the perfume) therein and applying the resultant slurry to the substrate from an applicator roll with which the substrate was brought into contact. Additional rolls were used to spread the slurry before it was cooled to ambient temperature to solidify the composition. Perfume was then sprayed on to the impregnated substrate to produce the final product.

No appreciable build up of product was noted on the processing equipment and the product demonstrated virtual freedom from flaking (i.e. a flaking grade of 9+) when it was folded. Similar results are obtained if the glycerol is replaced by 0.3 g diethylene glycol or by 0.3 g 1,2-propane diol.

### Examples 2-10

The following products, in accordance with the invention, are prepared (in parts by weight):

## Claims

1. A laundry additive product comprising a normally solid detergent composition comprising a solid matrix having a melting point greater than 30°C and less than 80°C, in which matrix is dispersed solid particles of size < 150 pm, said solid particles comprising from 5% to 50% by weight of the composition, said composition being in water releasable combination with a flexible sheet substrate, the weight ratio of said composition to said substrate lying in the range from 1:2 to 12:1 characterised in that said composition includes a liquid processing aid selected from polyols of MWt ≤ 180 and boiling point (at atmospheric pressure) of at least 100°C in an amount 0.5% to 5.0% by weight of the composition.

2. A laundry additive product according to Claim 1 wherein the polyol is selected from glycerol, diethylene glycol, 1,2-propane diol and 2-methyl propane 1,2-diol.

3. A laundry additive product according to either one of Claims 1 and 2 wherein the polyol is present in an amount of from 0.5% to 3.0% by weight of the composition.

4. A laundry additive product according to any one of claims 1-3 wherein said detergent composition is composed of an organic matrix comprising a mixture of a polyethylene glycol of MWT 4,000-10,000 and a primary CS-C22 aliphatic alcohol condensed with an average of from 4 to 30 moles of ethylene oxide, said matrix forming a solidified liquid phase in which are dispersed solid particles of a compound selected from: wherein each R' is a hydrophobic organic group containing alkyl chains, alkenyl chains, alkyl benzyl chains, alkyl phenyl chains, ether linkages, alkylene groups, alkenylene groups, ester linkages, or amide linkages totalling from 8 to 22 carbon atoms and which may additionally contain or be attached to a polyethylene oxide chain containing up to 20 ethoxy groups, m is a number from one to three provided that no more than one R' in a molecule can have more than 16 carbon atoms when m is 2 and no more than 12 carbon atoms when m is 3, R² is an alkyl or hydroxyalkyl group containing from 1 to 4 carbon atoms or a benzyl group, with no more than one R² in a molecule being benzyl and x is a number from 1 to 3, Y is selected from and Z is a water-soluble anion selected from halide, methosulphate, carboxylate, hydroxide, or nitrate, in a number to give electrical neutrality of the cationic component wherein X is wherein M is hydrogen or an alkali metal ion where n is from 1 to 6 wherein R is C₁―C₉ linear or branched alkyl
Y is S0₃M, COOH or COOM where
M is an alkali metal ion, or mixtures of any of a) to d).

## Patentansprüche

1. Wäschezusatzprodukt, umfassend eine normalerweise feste Detergenszusammensetzung, die eine feste Matrix mit einem Schmelzpunkt größer als 30°C und kleiner als 80°C enthält, in welcher Matrix feste Teilchen einer Größe < 150 um dispergiert sind, wobei diese festen Teilchen 5 bis 50 Gew.-% der Zusammensetzung ausmachen, und diese Zusammensetzung sich in in Wasser freisetzbarer Kombination mit einem biegsamen Blattsubstrat befindet, wobei das Gewichtsverhältnis der Zusammensetzung zu dem Substrat im Bereich von 1:2 bis 12:1 liegt, dadurch gekennzeichnet, daß die Zusammensetzung ein flüssiges Verarbeitungshilfsmittel ausgewählt aus Polyolen mit einem Molekulargewicht ≤ 180 und einem Siedepunkt (bei Normaldruck) von mindestens 100°C in einer Menge von 0,5 bis 5,0 Gew.-%, bezogen auf die Zusammensetzung, enthält.

2. Wäschezusatsprodukt gemäß Anspruch 1, worin das Polyol ausgewählt ist aus Glycerin, Diethylenglykol, 1,2₋Propandiol und 2-Methyl-propan-1,2-diol.

3. Wäschezusatzprodukt gemäß einem der Ansprüche 1 und 2, worin das Polyol in einer Menge von 0,5 bis 3,0 Gew.-%, bezogen auf die Zusammensetzung, vorhanden ist.

4. Wäschezusatzprodukt gemäß einem der Ansprüche 1 bis 3, worin die Detergenszusammensetzung aus einer organischen Matrix zusammengesetzt ist, welche ein Gemisch aus einem Polyethylenglykol vom Molekulargewicht 4000 bis 10 000 und einem'primären aliphatischen C8- bis C₂₂-Alkohol kondensiert mit durchschnittlich 4 bis 30 Mol Ethylenoxid enthält, wobei die Matrix eine verfestigte flüssige Phase bildet, in der feste Teilchen einer Verbindung dispergiert sind, die ausgewählt ist aus: worin jedes R' eine hydrophobe organische Gruppe ist, welche Alkylketten, Alkenylketten, Alkylbenzylketten, Alkylphenylketten, Etherbindungen, Alkylengruppen, Alkenylengruppen, Esterbindungen oder Amidbindungen mit insgesamt 8 bis 22 Kohlenstoffatomen enthält, und welche zusätzlich eine Polyethylenoxidkette mit bis zu 20 Ethoxygruppen enthalten oder an eine solche Gruppe gebunden sein kann, m eine Zahl von 1 bis 3 bedeutet mit der Maßgabe, daß nicht mehr als ein R' in einem Molekül mehr als 16 Kohlenstoffatome enthalten kann, wenn m 2 bedeutet, oder nicht mehr als 12 Kohlenstoffatome enthalten kann, wenn m 3 bedeutet, R² eine Alkyl- oder Hydroxyalkylgruppe mit 1 bis 4 Kohlenstoffatomen oder eine Benzylgruppe bedeutet, wobei nicht mehr als ein R² in einem Molekül eine Benzylgruppe ist, und x eine Zahl von 1 bis 3 bedeutet, Y ausgewählt ist aus und Z ein wasserlösliches Anion ausgewählt aus Halogenid, Methosulfat, Carboxylat, Hydroxid oder Nitrat in einer Zahl, um elektrische Neutralität des kationischen Bestandteils zu ergeben, bedeutet, worin X ist, worin M Wasserstoff oder ein Alkalimetallion bedeutet, worin n 1 bis 6 bedeutet, worin R eine geradkettige oder verzweigtkettige Cᵢ- bis Cg-Alkylgruppe bedeutet;
Y S0₃M, COOH oder COOM bedeutet, worin
M ein Alkalimetallion ist, oder Gemische aus beliebigen Verbindungen a) bis d).

## Revendications

1. Produit additif de blanchissage comprenant une composition détergente normalement solide comportant une matrice solide ayant un point de fusion supérieur à 30°C et inférieur à 80°C, des particules solides de granulométrie inférieures à 150 pm étant dispersées dans cette matrice, lesdites particules solides constituant de 5% à 50% en poids de la composition, ladite composition étant en combinaison éliminable à l'eau avec un substrat en feuille souple, le rapport pondéral de ladite composition audit substrat étant dans l'intervalle de 1:2 à 12:1, caractérisé en ce que ladite composition contient un auxiliare de traitement liquide choisi parmi les polyols de poids moléculaire inférieur ou égal à 180 et de point d'ébullition (sous la pression atmosphérique) au moins égal à 100°C, en une quantité de 0,5% à 5% en poids de la composition.

2. Produit additif de blanchissage selon la revendication 1, dans lequel le polyol est choisi parmi le glycérol, le diéthylène-glycol, le 1,2-propane-diol et le 2-méthylpropane-1,2-diol.

3. Produit additif de blanchissage selon l'une quelconque des revendications 1 et 2, dans lequel le polyol est présent en une quantité de 0,5% à 3,0% en poids de la composition.

4. Produit additif de blanchissage selon l'une quelconque des revendications 1 à 3, dans lequel ladite composition détergente est composée d'une matrice organique comprenant un mélange d'un polyéthylène-glycol de poids moléculaire 4 000- 10000 et d'un alcool aliphatique primaire en C₈―C₂₂, condensé avec une moyenne de 4 à 30 moles d'oxyde d'éthylène, ladite matrice formant une phase liquide solidifiée dans laquelle sont dispersées des particules solides d'un composé choisi parmi: dans laquelle chaque R' est un groupe organique hydrophobe contenant des chaînes alkyle, des chaînes alcényle, des chaînes alkylbenzyle, des chaînes alkylphényle, des liaisons éther, des groupes alkylène, des groupes alcénylène, des liaisons ester ou des liaisons amide, totalisant de 8 à 22 atomes de carbone, et qui peut en outre contenir, ou être fixée à, une chaîne de poly(oxyde d'éthylène) contenant jusqu'à 20 groupes éthoxy, m est un nombre de 1 à 3, à condition que pas plus d'un groupe R' dans une molécule puisse avoir plus de 16 atomes de carbone lorsque m est égal à 2, et pas plus de 12 atomes de carbone lorsque m est égal à 3, R² est un groupe alkyle ou hydroxyalkyle contenant de 1 à 4 atomes de carbone, ou un groupe benzyle, pas plus d'un gorupe R² dans une molécule étant un groupe benzyle, et x est un nombre de 1 à 3, Y est choisi parmi et Z est un anion hydrosoluble choisi parmi un halogénure, un méthylsulfate, un carboxylate, un hydroxyde ou un nitrate, en un nombre conférant au constituant cationique la neutralité électrique, dans laquelle X est dans lesquelles M est un hydrogène ou un ion de métal alcalin dans laquelle n est de 1 à 6 dans laquelle R est un groupe alkyle linéaire ou ramifié en C₁―C₉
Y est S0₃M, COOH ou COOM, où
M est un ion d'un métal alcalin, ou des mélanges de n'importe lesquels des composés a) à d).
